

## [54] ALUMINA CORE FOR CASTING DS MATERIALS

[56]

## References Cited

## U.S. PATENT DOCUMENTS

|           |        |                            |        |
|-----------|--------|----------------------------|--------|
| 3,248,241 | 4/1966 | Rifai .....                | 106/65 |
| 3,972,367 | 8/1976 | Gigliotti, Jr. et al. .... | 164/72 |
| 4,026,344 | 5/1977 | Greskovich .....           | 164/26 |
| 4,031,945 | 6/1977 | Gigliotti, Jr. et al. .... | 164/72 |

[75] Inventors: **Frederic J. Klug, Amsterdam; Wayne D. Pasco, Ballston Lake, both of N.Y.***Primary Examiner*—Francis S. Husar*Assistant Examiner*—K. Y. Lin*Attorney, Agent, or Firm*—Donald M. Winegar; Joseph T. Cohen; Charles T. Watts[73] Assignee: **General Electric Company, Schenectady, N.Y.**[21] Appl. No.: **839,981**[22] Filed: **Oct. 6, 1977**[51] Int. Cl.<sup>2</sup> ..... **B28B 7/30; B28B 7/34**[52] U.S. Cl. ..... **106/38.9; 106/38.8; 164/28; 164/41; 164/132; 249/175; 264/44; 264/221**[58] Field of Search ..... **164/36, 41, 44, 131, 164/132, 72, 28, 138; 106/41, 73.4, 65, 38.9; 249/175; 264/44, 62, 221**

## [57] ABSTRACT

An alumina core for investment casting directionally solidified eutectic and superalloy materials consists of a central portion which has porosity which is continuous throughout. The material of the central portion has a micro-structure which is characteristic of alumina grains which have undergone vapor phase transport action. An outer layer of alumina encompasses the central portion and in integral therewith and contains porosity which is discontinuous.

6 Claims, 7 Drawing Figures



Fig. 1.



Fig. 2.



Fig. 3.



Fig. 4.

## EFFECT OF GRAPHITE ON LINEAR SHRINKAGE



Fig. 5.

## EFFECT OF GRAPHITE ON FIRED DENSITY

- MOLE %  $MgO$ -FAST HEATING RATE
- △ 15 MOLE %  $MgO$ -FAST HEATING RATE
- ▲ 15 MOLE %  $MgO$ -SLOW HEATING RATE



Fig. 6.

WEIGHT LOSS DUE TO REACTION  
BETWEEN GRAPHITE & ALUMINA

## MOLAR RATIO

- $G/A = 0$
- $G/A = 0.25$
- $G/A = 0.75$
- △  $G/A = 1.25$



Fig. 7.

EFFECT OF GRAPHITE  
ON FIRED DENSITY

**ALUMINA CORE FOR CASTING DS MATERIALS****RIGHTS GRANTED TO THE UNITED STATES  
OF AMERICA**

The Government of the United States of America has rights in this invention pursuant to Contract No. F33615-76-C-5110 awarded by the Department of the Air Force.

**BACKGROUND OF THE INVENTION****1. Field of the Invention**

This invention relates to improvements in investment casting and in particular to a new and improved alumina core for employment therewith.

**2. Description of the Prior Art**

The production of directionally solidified (DS) metal eutectic alloys and superalloys for high pressure turbine (HPT) airfoils with intricate internal passageways for air cooling requires that the core and mold not only be dimensionally stable and sufficiently strong to contain and shape the casting but also be sufficiently weak to prevent mechanical rupture (hot cracking) of the casting during solidification and cooling. The DS process requirements of up to 1875° C for a 16 hr. time period imposes severe constraints on materials which may serve as mold or core candidates.

The prior art appears to be mostly limited to the use of silica or silica-zircon core and mold materials. At temperatures greater than 1600° C the silica based materials fail from the standpoint of both mechanical integrity and chemical incompatibility with the advanced alloy compositions.

Dimensional control of the silica core is excellent since cristobalite exhibits very little densification. Microstructural examination reveals that, in some cases, commercial core compositions employ very large particles ( $>100\mu\text{m}$ ). The addition of large particles serves to lower both shrinkage and mechanical strength.

Paul S. Svec in "Process For Making an Investment Mold For Casting And Solidification of Superalloys Therein", U.S. Patent application Ser. No. 590,970, teaches the use of alumina-silica compositions for making molds and cores. Charles D. Greskovich and Michael F. X. Gigliotti, Jr. In U.S. Pat. Nos. 3,955,616 and 3,972,367 teach cores and molds of alumina-silica compositions which have a barrier layer of alumina formed at the mold/metal interface. One possible means for the formation of their alumina layer is by a chemical reaction wherein carbon of the susceptor chemically reduces the material composition of the mold or core. Charles D. Greskovich in U.S. Pat. No. 4,026,344 also teaches an alumina-silica composition wherein the material is of a predetermined size so as to favor, and therefore enable, the formation of metastable mullite for molds and cores which exhibit superior sag resistance at high temperatures.

Aluminum oxide by itself, without a chemical or physical binder material, has been identified as a potential core and mold material based on both chemical compatibility and leachability considerations. There is, however, a considerable thermal expansion mismatch between the ceramic and the alloy which generates, around the ceramic core, hoop and longitudinal tensile stresses in the alloy on cooling from the DS temperature. The high elastic modulus and high resistance to deformation at elevated temperatures of dense alumina and its lower coefficient of thermal expansion than the

alloy result in the mechanical rupture or hot tearing of the alloy.

A mechanism by which an alumina core body can deform under the strain induced by the cooling alloy must be developed to permit the production of sound castings. The microstructure of the ceramic core and mold must be tailored to permit deformation under isostatic compression at a stress low enough to prevent hot tearing or cracking of the alloy. The surface of the core and mold must also serve as a barrier to metal penetration. It would be highly desirable to have a core wherein a central portion would have continuous porosity and good crushability characteristics. A barrier layer having discontinuous porosity should encompass, and be integral with, the central portion of the core. Such a core must also be easily removed from the casting with minimum effort and little effect on the quality of the cast metal.

An object of this invention is to provide a new and improved core for casting directionally solidified eutectic and superalloy materials having superior porosity and crushability characteristics than prior art cores.

Another object of this invention is to provide a new and improved core for casting directionally solidified eutectic and superalloy materials wherein the material of a central portion thereof has a porous microstructure and the grain morphology is characteristic of grains which have undergone vapor phase transport action and a dense layer of alumina, wherein the porosity is discontinuous, encompasses and is integral with the central portion.

Other objects of this invention will, in part, be obvious and will, in part, appear hereinafter.

**BRIEF DESCRIPTION OF THE INVENTION**

In accordance with the teachings of this invention there is provided a new and improved alumina core for use in the investment casting of directionally solidified eutectic and superalloy materials. The core comprises an outer portion which encompasses and is integral with a central portion. The material of the outer portion is dense and any porosity therein is discontinuous. The material of the inner portion has a porous microstructure of alumina whose grain morphology is characteristic of grains which have undergone vapor phase transport action. The porosity is continuous throughout the central portion of the core. The vapor transport action results in a network of narrow connecting bridges between the alumina particles.

**DESCRIPTION OF THE DRAWINGS**

FIG. 1 is a photomicrograph of a portion of a fired compact of alumina. (50x)

FIG. 2 is a scanning electron micrograph at 500x of the compact of FIG. 1 showing the morphology of the alumina grain structure.

FIG. 3 is a plot of Log of the leaching rate versus theoretical density of a fired alumina compact.

FIG. 4 is a plot showing the effect of graphite additions on the linear shrinkage of a fired alumina compact.

FIG. 5 is a plot showing the effect of graphite additions on the density of a fired alumina compact.

FIG. 6 is a plot showing the weight loss due to the reaction between graphite and alumina in a fired compact.

FIG. 7 is a plot showing the effect of graphite on the density of a fired compact.

## DESCRIPTION OF THE INVENTION

With reference to FIGS. 1 and 2 there is shown a portion of a compact 10 made from an alumina ceramic material composition embodying a reactant fugitive filler material. The compact 10 is made of alumina material fired in a controlled atmosphere to form a layer 12 of alumina as an outer portion encompassing and integral with a central portion 14 of alumina. The alumina of the layer 12 is dense, that is, any porosity therein is discontinuous. The structure of the material of the central portion 14 is porous and the porosity is continuous throughout.

As better illustrated with reference to FIG. 2, the microstructure of the central portion 14 of the fired compact 10 has a porosity which is continuous throughout. Additionally, examination of the alumina grains 16 clearly indicates a grain morphology which is characteristic of alumina grains which have undergone vapor phase transport action. The vapor transport action involves the evaporation and/or formation of a gaseous suboxide of a portion of material of one grain at high surface energy regions of the grain and the transportation of the material to low surface energy regions of the grain where it condenses or is oxidized. By this action the alumina grains 16 become coarse and rounded. Additionally, aluminum suboxide gaseous species are transported away from the center portion 14 of the compact 10 where at least some of the species is oxidized at the outer surface thereof to form the integral outer portion 12 of alumina. As a result of the chemical reaction producing this vapor transport action, the fired compact registers a weight loss. Further, the vapor transport action results in a network of narrow connecting bridges 18 between the alumina particles or grains 16.

The compact 10 is suitable for use as a core in investment casting of directionally solidified eutectic and superalloy materials. It is desirable for the cooling passages of the turbine blade to have a complex configuration. Therefore, it is necessary for the compact or core to have a complex shape. The preferred method of forming the compact or core 10 in an unfired state is by injection or transfer molding. The preferred material for the compact or core 10 is alumina or magnesia doped alumina because casting temperatures are in excess of 1600° C and as high as 1850° C while directional solidification times are in excess of 16 hours.

The alumina compact 10 is easily removed from the casting by leaching in a KOH or NaOH solution in an autoclave. The leaching rate, however, is dependent upon the porosity of the compact 10. As shown in FIG. 3, if one can manufacture a compact 10 with a porosity content of from 60 percent to 70 percent by volume, a very significant increase in the leaching rate of the compact 10 can be obtained. Additionally, the compact 10 would make an acceptable core for making turbine blades wherein the wall thickness is about 0.060 inch or less since it will have good crushability characteristics.

In injection molding, the solids content of the material composition employed to form a compact to function as a core, and having a complex shape, initially must be in excess of 50 percent by volume to prevent the solids included therein from becoming a discontinuous phase. Should the solid material become a discontinuous phase upon binder removal and before sintering occurs, the compact may deform or disintegrate.

To increase porosity in the fired compact a reactant fugitive filler material is desirable. The reactant fugitive

filler material provides, along with the alumina material, the total solids content necessary for injection molding. Upon a subsequent firing at an elevated temperature, the reactant fugitive filler is "burned" off in a suitable manner to increase the porosity content of the compact 10. A desirable reactant fugitive filler material is one which will also react with the alumina to eliminate or remove a portion thereof from the compact 10 and thereby increase the porosity content further. Suitable fugitive filler materials are those which will provide enough reactant material at the elevated temperature to reduce a portion of the alumina which, in part, is removed from the compact in the gaseous state and which, in part, is either deposited on other alumina grains by vapor phase transport action causing a coarsening and a rounding thereof or oxidized to form the integral outer portion 12 of alumina. Preferred reactant bearing materials are graphite, aluminum, aluminum carbide, aluminum oxycarbide, boron and boron carbide. Suitable organic materials may also be employed as reactant materials as a carbon source.

The particle size of the alumina is important. It is desirable that the size of the pores in the compact, particularly at the outside surfaces which contact the cast metal, be small enough to prevent any significant metal penetration. It is desirable that metal penetration of the compact surface be minimized in order to obtain the best surface possible for the casting. The integral outer portion 12 of alumina functions as a barrier layer to prevent metal penetration into the core structure. The particle size distribution of the alumina has a significant effect on the rheology of the wax-carbon-alumina systems. The alumina or magnesia doped alumina and the carbon bearing material should have a particle size of less than 300 microns. The preferred particle size range is from 1-50 microns.

Suitable alumina material is obtainable as fused alumina powder from the Norton Company and as aggregate free alumina powder from the Meller Company. Suitable alumina powders are

(a) Norton-400 Alundum wherein the particle size distribution is typically as follows:

| Particle Size       | Weight percentage |
|---------------------|-------------------|
| 0 - 5 $\mu$         | 15%               |
| 5 $\mu$ - 10 $\mu$  | 13%               |
| 10 $\mu$ - 20 $\mu$ | 64%               |
| 20 $\mu$ - 30 $\mu$ | 7%                |
| > 30 $\mu$          | 1%                |

(b) Norton-320 Alundum where in the particle size distribution is typically as follows:

| Particle Size       | Weight percentage |
|---------------------|-------------------|
| 0 - 10 $\mu$        | 3%                |
| 10 $\mu$ - 20 $\mu$ | 53%               |
| 20 $\mu$ - 30 $\mu$ | 36%               |
| 30 $\mu$ - 37 $\mu$ | 7%                |
| > 37 $\mu$          | 1%                |

(c) Norton 38-900 Alundum wherein the particle size distribution is typically as follows:

| Particle Size      | Weight percentage |
|--------------------|-------------------|
| 0 - 5 $\mu$        | 55.5              |
| 5 $\mu$ - 10 $\mu$ | 34.0              |
| > 10 $\mu$         | remainder         |

(d) Meller 0.3 $\mu$  aggregate free alumina

Various possible ceramic mixtures include 80 weight percent Norton-400, balance Meller 0.3 $\mu$ ; 70 weight percent Norton-400, balance Meller 0.3 $\mu$ ; 100 weight percent Norton-320; 80 weight percent Norton-320, balance Norton 38-900, and 100 weight percent Norton 38-900.

Alumina doped with at least 1 mole percent magnesia is also suitable as a ceramic material for making the compact 10. It is believed that the addition of the divalent alkaline earth cations into the trivalent cation lattice of  $Al_2O_3$  introduces lattice defects which enhance the kinetics of the dissolution of alumina during autoclave caustic leaching.

The magnesia may be present in amounts from about 1 mole percent up to about 30 mole percent. It has been discovered that as the magnesia content decreases, the volume fraction of the magnesia doped alumina phase increases. The magnesia doped alumina phase encases the spinel phase. The spinel phase therefore provides either an interconnected network defining a plurality of interstices in which the magnesia doped phase is found or a dispersion of particles within a matrix of magnesia doped alumina.

Above about 20 mole percent magnesia, the magnesia doped alumina network begins to become discontinuous. Dissolution of the alumina network by autoclave KOH or NaOH processing therefore begins to require an excessive increase in processing time. The decrease in dissolution is attributed to the fact that autoclave leaching must occur by intergranular attack which at a magnesia content of about 25 mole percent is almost an order of magnitude slower than at 20 mole percent content.

Two methods of fabricating compacts with magnesia doped alumina may be employed. In one instance a mechanical mix of alumina powder of the desired particle size content and the appropriate amount of magnesia is prepared. This mechanical mixture is then added to the melted wax.

In the second instance, the same mechanical mixture is prepared and calcined at a temperature of  $1500^\circ C \pm 200^\circ C$  for about 1 to 4 hours to form a two phase product of spinel and magnesia doped alumina. The calcined product is then crushed and ground to a particle size of from 1 $\mu$ m to 40 $\mu$ m. This mechanical mixture is then added to the melted wax.

One or more waxes can be employed to provide adequate deflocculation, stability and flow characteristics. The plasticizing vehicle system preferably consists of one or more paraffin type waxes which form the base material. A purified mineral wax ceresin may also be included in the base material. To 100 parts of the base wax material additions of oleic acid, which acts as a deflocculant, white beeswax, which acts as a deflocculant and aluminum stearate, which acts to increase the viscosity of the base wax, are added. A preferred plasticizing vehicle has the following composition:

| Binder:                           | Material | Part By Weight   |           |
|-----------------------------------|----------|------------------|-----------|
| P-21 paraffin (Fisher Scientific) |          | 33 $\frac{1}{3}$ |           |
| P-22 paraffin (Fisher Scientific) |          | 33 $\frac{1}{3}$ |           |
| Ceresin (Fisher Scientific)       |          | 33 $\frac{1}{3}$ |           |
| Total                             |          | 100 parts        |           |
| Part By Weight                    |          |                  |           |
| Additives:                        | Material | Range            | Preferred |
|                                   |          |                  | Typical   |
| oleic acid                        | 0-12     | 6-8              | 8         |
| beeswax,                          | 0-12     | 3-5              | 4         |

-continued

|                               |      |     |   |
|-------------------------------|------|-----|---|
| white<br>aluminum<br>stearate | 0-12 | 3-6 | 3 |
|-------------------------------|------|-----|---|

Despite the addition of deflocculant, large particle size, of the order of  $>50\mu$ , can settle at a rather rapid rate in the wax and can change the sintering behavior of the remainder of the material mix of the molding composition material. The rate of settling of large particles is adjusted by varying the viscosity of the liquid medium, wax. To this end aluminum stearate is added to the wax to increase viscosity by gelling. Increased viscosity also has the additional benefits of preventing segregation of the wax and solids when pressure is applied and reducing the dilatancy of the material mixture.

In order to describe the invention more fully, and for no other reason, the reactant fugitive filler material is said to be a carbon bearing material. The amount of carbon bearing material added to the core composition mix is dependent upon the porosity desired in the fired core as well as the average particle size of the alumina material. The carbon material present in the core material mix as graphite has a molar ratio of carbon to alumina of from about 0.3 to 1.25. This molar ratio range has been found to provide excellent results. The graphite is retained in the bisque ceramic during heating until the alumina begins to sinter and develops strength at the alumina-alumina particle contacts. The graphite can now be removed from the structure, or compact, without producing a discontinuous solid phase that could cause distortion of the compact.

The expected chemical reactions between alumina and carbon occur at temperatures greater than  $1500^\circ C$  in a reducing or inert atmosphere. The result of these reactions is the production of volatile suboxides of alumina. The possible reactions are:



with (2) being the most probable reaction to occur.

At temperatures above  $1500^\circ C$ , the vapor pressure of the suboxide is significant. As the vapor pressure increases, mass transport by an evaporation-condensation type mechanism can occur. If the rate of mass transport through the vapor phase is much greater than mass transport by volume or grain boundary diffusion, the material is merely rearranged in the compact and no reduction in the pore volume (i.e. densification) can take place. In the reducing or inert atmosphere, the suboxide can escape thereby lowering the density of the compact or fired ceramic and producing the microstructure of the central portion 14 of the compact 10 as illustrated in FIGS. 1 and 2.

The effect of carbon additions, in the form of graphite, on the weight loss of the ceramic article when fired in a reducing atmosphere, such as hydrogen, is a function of the heating rate and the atmosphere above about  $900^\circ C$ .

When the heating rate is less than the order of about  $100^\circ C$  per hour in the temperature range of from about  $900^\circ$  to about  $1500^\circ C$ , with oxygen present as an impu-

rity in the controlled atmosphere, the expected porosity content is not obtained. Apparently, the carbon reacts with the gaseous oxygen impurity to form gaseous CO and CO<sub>2</sub>, which escapes from the compact. Consequently, insufficient carbon is available above about 1500° C to reduce the alumina to a gaseous suboxide and produce the fired compact of desired porosity content.

Controlled atmospheres for firing the compact and to obtain the desired chemical reactions in the remaining material may be of a reducing type or of an inert gas type. Hydrogen may be employed as a reducing gas type atmosphere. Argon, helium, neon and the like may be utilized for atmospheres of the inert gas type.

As shown in FIG. 4 the effects of carbon additions on the linear shrinkage of the fired ceramic is dependent upon the molar ratio of carbon to alumina, the amount of oxygen impurity in the atmosphere, and the heating rate.

As the molar ratio of carbon to alumina is increased the percent linear shrinkage of the compact is decreased. The molar ratio of carbon to alumina may be inadvertently reduced in the compact during the firing if oxygen impurities in the atmosphere react with a portion of the carbon in the compact to form CO or CO<sub>2</sub>. In FIG. 4, the effect of the heating rate on the oxidation of carbon is shown. When a slow heating rate is employed, the carbon to alumina ratio is lowered by oxidation of carbon and high shrinkages result. When a fast heating rate is used the carbon to alumina ratio is not greatly affected by oxidation of carbon and low shrinkages result. If the firing atmosphere were completely free of any oxygen or water vapor the resulting linear shrinkage would be independent of the heating rate used and would only be a function of the initial carbon content. For example, when the carbon to alumina ratio is about 0.75, the linear shrinkage is only 2% if a fast heating rate is practiced when the controlled atmosphere includes the presence of oxygen as an impurity therein. In contrast, under the same conditions, with a slow heating rate, a linear shrinkage as high as 13% has been observed. A low shrinkage is desirable in producing the required close dimensional tolerances. The same effects are noted when undoped or pure alumina flour is employed in the core composition mix.

The percent linear shrinkage is also dependent on the grain size of the alumina flour employed. A larger grain size material will decrease the percent linear shrinkage which will occur. Therefore, as stated previously, the grain size of the alumina flour employed in making the fired compact 10 is preferably from about 1 micron to about 50 microns.

Referring now to FIG. 5, the molar ratio of carbon to alumina and of carbon to magnesia doped alumina affects the density of the fired core. An increasing molar ratio of up to 0.75 results in decreasing the fired density of the ceramic article to about 40 percent of full density from an initial 70 percent of full density when practiced at a fast heating rate with an oxygen impurity present. However, when a slow heating rate is practiced in the presence of oxygen impurity, the percentage of full density for an article embodying a carbon to magnesia doped alumina of from 0 to 0.75 remains almost at approximately 70 percent.

Although the molar ratio of carbon (with the carbon expressed as graphite) to alumina affects the various physical characteristics of the fired ceramic articles, the rate of heating concomitant with the oxygen partial pressure also has a pronounced effect on the fired arti-

cles. Therefore, an improperly fired ceramic article has less porosity, exhibits poorer crushability characteristics, undergoes higher shrinkage and requires a longer leaching time to remove the ceramic article from the casting.

With reference to FIG. 6, the percent weight loss due to the loss of carbon and/or alumina is dependent upon the firing temperature. Above about 1550° C, the loss becomes appreciable and is related to molar ratio of carbon to alumina. The greater effect is noted when the molar ratio is of the order of 0.75 and above.

Referring now to FIG. 7, the effect of the molar ratio of graphite to alumina on the fired density of ceramic articles made from the material composition mix of this invention is shown. For molar ratios of 0.25 to 0.75, the fired density increases slightly with increasing temperature up to about 1500° C. Above 1500° C, the higher molar ratio materials shows a significant decrease in the fired density of the ceramic article.

The following teachings of this invention reveal the effects of the dewpoint of the hydrogen gas. Equivalent partial pressures of oxygen in inert gases can also be employed to form the desired structure of the fired compacts. However, for purposes of illustration only, and for no other reason, the invention is further described employing hydrogen gas having a given dewpoint range.

In order to form the outer portion 12 of alumina while achieving the desirable microstructure of the inner portion 14, the compact 10 is fired at the elevated temperature of about 1500° C and upwards in an atmosphere of controlled dewpoint hydrogen gas. The wet hydrogen gas has a dewpoint of from about -5° F to no greater than about +25° F. Preferably, the dewpoint of the hydrogen gas should be greater than about 0° F. Suitable inert gases are argon, helium, neon and the like containing the desired partial pressure of oxygen.

It is preferred not to have the dewpoint exceed +25° F since the compact undergoes less of a weight loss and the reaction times become increasingly longer with increasing dewpoint values above about +25° F. This may be occurring as a result of the following reaction between water of the wet hydrogen gas and the reactant fugitive material carbon



wherein an increase in the amount of H<sub>2</sub>O available for reacting with the carbon causes the compact to lose greater amounts of carbon through oxidation.

The outer portion 12 has a thickness which may vary from 5 microns or less to about 100 microns. The firing temperature has a range of from 1650° to about 1900° C with a preferred range of from about 1750° to about 1850° C. The compact is fired in this range for a period of from about 15 minutes to about 4 hours in order to achieve the range of thickness of the outer portion 12.

Other suitable alumina starting materials may include rare earth doped alumina wherein the alumina is in excess and the reactant fugitive filler material will reduce the excess alumina present. Such materials include yttrium aluminate and lanthanum aluminate.

The composition of this invention when prepared for injection molding may be prepared in several ways. A preferred method embodies the use of a Sigma mixer having a steam jacket for heating the contents. When the plasticizer material is comprised of one or more waxes, the wax is placed in the mixer and heated to a

temperature of from 80° to 110° C to melt the wax or waxes. The additive agents of one or more deflocculents and aluminum stearate are then added, as required, in the desired quantities. The mixing is continued for about 15 minutes to assure a good mixture of the ingredients. The desired quantity of reactant fugitive filler material is then added and mixing, at the elevated temperature, is continued until all visible chunks of reactant fugitive filler material are broken up. To this mixture is then added the alumina bearing flour or mixture of flours of the desired size distribution. Mixing is then continued, in vacuum, at the elevated temperature for about 30 minutes or until the flour materials are universally distributed throughout the mixture. The heat is turned off and coolant water passed through the steam jacket to cool the mixture. Mixing is continued for a period of from 30 to 40 minutes, or until the mix is pelletized to a desired size of less than 2 cm.

Employing the composition mix of this invention one is able to injection mold complex shaped cores at from 200 psi to 10,000 psi and upwards to 50,000 psi at temperatures of from 80° to 130° C. The shrinkage rate of such composition mix is on the order of about 1 percent by volume.

The wax is removed from the pressed compact by heating the compact to a temperature of several hundred degrees Celsius until the wax or plasticizer material drains from the compact. Preferably, the pressed compact is packed in fine alumina or carbon flour having a finer pore size than the pore size of the pressed compact after wax removal. This enables the wax to be withdrawn by a capillary action induced by the finer pore size packing material. Other suitable packing materials are activated charcoal, high surface area carbon black and activated alumina. The wax, as described heretofore, is almost completely removed from the pressed compact at about 200° C. Subsequent heat treatment is used to sinter the compact or core material to increase its mechanical strength for handling purposes.

A typical heating cycle may include a rate of heating at about 25° C per hour from room temperature up to about 400° C to remove any wax still present in the compact. Thereafter the heating rate practiced is from about 50° C per hour to about 100° C per hour up to a temperature range of from 1100° C to 1300° C.

The core, or compact 10, is removed from the packing material and extraneous carbon is removed from the outside surfaces thereof by suitable means such as brushing. Thereafter; the core, or compact, is heated at a rate of 100° C per hour or greater.

Preferably above about 1300° C, the heating rate is increased until it is greater than about 200° C per hour and is practiced up to an elevated temperature of about 1650° C or greater, depending upon the end use of the compact, or core. Upon reaching the elevated temperature, isothermal heating is practiced for a sufficient time for the carbon available to react with the alumina present to produce the desired level of porosity in the fired core.

An alternate heating or firing schedule entails a partial removal of the wax from the compact by heating the compact at less than 25° C/hr to a temperature of no greater than 200° C in packing material. The wax remaining is only of the order of from 2% by weight to 4% by weight. The compact is then removed from the packing powder and placed in the sintering furnace. The wax still remaining in the compact gives the compact good handling strength. A heating rate of less than

25° C per hour is employed up to about 400° C to remove the remainder of the wax. In order to avoid any oxidation of the reactant fugitive filler material, the subsequent heating rate should be as rapid as possible.

5 The compact is thereafter heated at a rate greater than 200° C per hour up to 1650° C or higher depending on the end use of the compact. Upon reaching this predetermined elevated temperature, isothermal heating is practiced for a sufficient time for the reactant fugitive filler material to react with the alumina present to produce the desired level of porosity in the compact.

Any excess carbon in the fired compact is removed by heating the fired compact in an oxidizing atmosphere at a temperature greater than 900° C. Unbound carbon should be removed from the fired compact to prevent possible "boiling" of the cast metal during the practice of solidification of eutectic and superalloy materials.

Gaseous suboxides of alumina form in a reducing atmosphere above about 1500° C to form the desired porous microstructure of the compact 10. The outer barrier region 12 which consists of a dense continuous layer of alumina is formed by oxidation of a portion of the aluminum suboxide at the surface of the compact 10. The remainder of the gaseous suboxides which are not employed in forming the barrier layer 12 escape from the compact 10 into the furnace atmosphere. The formation of the dense continuous barrier layer 12 occurs at dewpoints of greater than -5° F in hydrogen concomitant with a furnace temperature of greater than 1550° C. The preferred condition for formation of a dense continuous barrier layer 12 is a dewpoint of from about +0° F to about +25° F for hydrogen gas, and the equivalent range of partial pressure of oxygen in a suitable inert gas, concomitant with a furnace temperature range of from about 1750° to about 1850° C.

It is significant to note that when the gases of the controlled atmosphere are completely free of oxygen or water vapor, the heating rate is of little or no importance.

When the fugitive reactant material is either aluminum or boron, the probable chemical reactions between alumina and aluminum and boron, include the following:



To illustrate the capability of either boron or aluminum to function as a reactant fugitive filler material, material compositions of alumina and reactant fugitive filler material were prepared. The molar ratio of reactant fugitive filler material to alumina was 1:2. The material compositions were mechanically mixed and pressed into pellets having a density of about 60% of theoretical. The pellets were then fired in hydrogen, dewpoint -33° F, and heated to an elevated temperature of 1765° C ± 20° C at a rate of 1300° C/hr. The pellets containing aluminum as a reactant fugitive filler material were isothermally heated at temperature for a period of 1 hour. The pellets containing boron as a reactant fugitive material were isothermally heated at temperature for a period of 30 minutes. The pellets were removed from the furnace and cooled to room temperature and then examined.

The pellets having aluminum as a reactant fugitive material registered a weight loss of about 20 percent. The pellet density was about 63 percent of theoretical density. The pellets having boron as a reactant fugitive material registered a weight loss of about 22 percent. The density of the pellets was about 45 percent theoretical.

The teachings of this invention have been directed towards compacts employed as cores having a complex shape wherein metal cast about the core has a wall thickness of the order of 0.060 inch or less. Therefore, "hot cracking" is critical. When the wall thickness of the cast metal is greater, less porosity is required as the metal has strength to resist the forces exerted by the core. In such instances porosities less than 50 percent by volume can be tolerated. Therefore, compacts for such cores may be prepared with smaller amounts of the reactant fugitive filler. Compacts of simple shapes can be made by simple compaction and subsequent firing following most of the heating sequences described heretofore for compacts including a wax binder. The compact may comprise an alumina bearing flour of the desired particle size range and a reactant fugitive filler to produce the desired porosity content.

We claim as our invention:

1. A core suitable for use in investment casting comprising a shaped body of ceramic material including a central portion and an integral outer portion enclosing the central portion therein,

5

10

15

20

25

30

the ceramic material of the central portion is characterized by a porous microstructure, wherein the porosity content is greater than 20 percent by volume, and is characteristic of grains which have undergone vapor phase transport action, and the ceramic material of the integral outer portion is characterized by a dense layer of the same ceramic material as that of the central portion.

2. The ceramic article of claim 1 wherein the ceramic article comprises alumina.
3. The ceramic article of claim 1 wherein the porosity content of the central portion is greater than 50 percent by volume, and is continuous throughout the body, the porosity in the integral outer portion is characterized by a dense layer of ceramic material wherein the porosity is discontinuous, and further including a network of narrow connecting bridges of ceramic material interconnecting adjacent particles in the central portion.
4. The ceramic article of claim 3 wherein the ceramic material of the body comprises alumina.
5. The ceramic article of claim 4 wherein the alumina is doped with from 5 mole percent to 15 mole percent magnesia.
6. The ceramic article of claim 2 wherein the alumina is doped with from 5 mole percent to 15 mole percent magnesia.

\* \* \* \* \*

35

40

45

50

55

60

65